

# United States Patent [19]

Schwarz

[11] 3,899,341

[45] Aug. 12, 1975

[54] **REFRACTORY FIRED SHAPED ELEMENT  
AND PROCESS OF ITS MANUFACTURE**

[75] Inventor: **Hans Georg Schwarz**, Marktredwitz,  
Germany

[73] Assignee: **Didier-Werke AG**, Germany

[22] Filed: **Apr. 4, 1974**

[21] Appl. No.: **458,022**

|           |         |                     |        |
|-----------|---------|---------------------|--------|
| 2,593,352 | 4/1952  | Shaw et al. ....    | 106/57 |
| 2,624,097 | 1/1953  | Kistler.....        | 106/57 |
| 3,175,919 | 3/1965  | Smoot et al. ....   | 106/57 |
| 3,228,778 | 1/1966  | Walther et al. .... | 106/57 |
| 3,620,781 | 11/1971 | Garvie .....        | 106/57 |

*Primary Examiner*—J. Poer  
*Attorney, Agent, or Firm*—Wenderoth, Lind & Ponack

[30] **Foreign Application Priority Data**

Apr. 30, 1973 Germany..... 2321810

[52] **U.S. Cl. .... 106/57**

[51] **Int. Cl.<sup>2</sup> .... C04B 35/48**

[58] **Field of Search**..... 106/57

[56] **References Cited**

UNITED STATES PATENTS

2,553,265 5/1951 Mochel..... 106/57

[57]

## ABSTRACT

Novel refractory-fired, shaped elements for closures in pouring units for steel, iron and metal (nozzles, stoppers, spouts, slides) are provided. Said elements are based on zirconium oxide and zirconium silicate. The elements have advantageous thermal and mechanical properties and are economical to produce. A novel process for the production of these elements is also provided.

6 Claims, No Drawings

**REFRACTORY FIRED SHAPED ELEMENT AND  
PROCESS OF ITS MANUFACTURE**

The invention relates to refractory-fired, shaped elements for closures in pouring units for steel, iron and metal (nozzles, stoppers, spouts, slides), said elements being based on zirconium oxide and zirconium silicate and a process for their manufacture.

Refractory closures are employed in connection with pouring the molten steel from ladles. Such closures are situated in or on the pouring units. The task of such refractory closures is to maintain, as constant as possible, the amount of steel flowing out therethrough per unit of time, in order to optimize the subsequent solidification and cooling process. The amount of steel flowing out per unit of time is substantially a function of the level of the steel bath in the casting unit and of the cross section of the opening of the closure.

Accordingly, the closures are subjected to rigorous requirements in regard to the resistance to wear, in relation to the steel, iron or metal flowing therethrough high temperatures, and particularly in regard to resistance to deterioration as a result steep changes of temperatures, since the pouring units provided with the above-mentioned closures are filled automatically with highly-heated, fused material (steel, iron and metal). To combat such high stress, zirconium silicate ( $ZrSiO_4$ ) has been already employed as material for manufacturing closing parts, e.g., nozzles. However, the possibilities of employing nozzles of zirconium silicate are limited. The difficulties associated with zirconium silicate nozzles result during long casting periods and while casting rimmed or alloyed steels. The severe stress manifests itself in the noticeable widening of the cross section of the nozzle opening, which leads to an uncontrolled variation in the rate of pour. Previous attempts to remedy this problem included employment of closures made of zirconium oxide or dense aluminum oxide. However, wide application of such products is prevented by the price of the material, which is very high in comparison with the products of zirconium silicate, and, most importantly, by a high sensitivity to thermal shock, which is found in such products.

Experiments employing mixtures of zirconium oxide and zirconium silicate as starting material for refractory bricks have also been made. Thus, Harders-Kienow, in their book, "Feuerfestkunde", pages 906-7 (1960), Springer-Verlag proposed to employ a mixture of 1000 g zirconium oxide and 500 g zirconium silicate (66.66 % by weight  $ZrO_2$  and 33.34 % by weight  $ZrSiO_4$ ) for making light refractory bricks. However, the employed brick is employed only for the purpose of insulation. Due to its high porosity, it cannot be employed as shaped element for closures of casting units which transmit the flow of fused steel. On the contrary, a shaped element for pouring purposes must be dense in order to resist effectively the corrosion.

The invention is based on the task of developing a reasonably priced, quality zirconium-based material for shaped elements to be inserted into closures in casting units for steel, iron and metal, which encompasses the advantages of a high resistance to wear and to a high resistance in regard to thermal shocks.

The problem is solved by employing a composition comprising zirconium oxide at 10-50 % by weight, preferably 35 % by weight, zirconium silicate at 50-90 % by weight, preferably 65 % by weight. Moreover, 30

-60 % by weight of the entire amount of zirconium oxide present must be in stabilized form and 70-40 % by weight must be in a non-stabilized form. The zirconium oxide is employed in a grain size of at most 0.1 mm, and preferably smaller than 0.06 mm, and the zirconium silicate is introduced in a grain size exceeding 0.2 mm, preferably 0.2-0.5 mm.

The portion of zirconium oxide (grain size under 0.1 mm, preferably smaller than 0.06 mm) is based on the idea of introducing this valuable material only in an amount required for a good resistance to corrosion. In the completed brick, this corrosion-resistant material forms the matrix, due to its fine grains, which matrix is resistant to slag corrosion.

15 The employment of inexpensive zirconium silicate in an amount of 50-90 % by weight, preferably 60 % by weight of the mixture, secures a price advantage in relation to materials possessing the same durability. This material, which is more susceptible to slag-corrosion then zirconium oxide, is made similar to that of zirconium oxide through its employment in the form of coarse grains (0.2-0.5 mm).

20 The composition of the invention, zirconium silicate in coarse grains, zirconium oxide in fine powder, produces a fired element with a framework of zirconium silicate comprising an intermediate matrix of sintered zirconium oxide. Since the known dissociation of the  $ZrSiO_4$  at high temperatures



proceeds from the inner surface, the fraction of silicic acid released through decomposition in the composition of the mixture of the invention ( $ZrSiO_4$  being in coarser grain) is smaller by a multiple than the fraction 35 corresponding to the quantitative substitution of the  $ZrSiO_4$  in the mixture by  $ZrO_2$ . This again leads to the fact that the matrix contains a smaller amount of low-melting compounds and, consequently, is much more effective against the corrosive action at high temperature. Moreover, the  $ZrSiO_4$  framework confers a good stability in relation to the variation of temperature to the fired product.

40 The zirconium oxide to be added in accordance with the invention is a material that in its original modification, exhibits reversible changes of volume at increased temperature (above 1000°C), which leads to cracks in the structure of a mass which contains this material in excess. This disadvantage is avoided by employing stabilized zirconium oxide. In order to avoid the introduction of fluxing materials into the matrix of zirconium oxide beyond a certain extent and the resulting detrimental effect exerted on its refractory properties, the addition of stabilized zirconium oxide, containing  $CaO$  as stabilizer (as is well known), is quantitatively limited.

45 The upper limit of the additive is situated at about 60 % by weight of the entire zirconium-oxide material. On the other hand, there is required a minimum amount, in order to obtain the stabilizing effect in the mixture 50 (minimum amount: 30 % by weight of the amount of zirconium oxide).

55 The shaped elements are manufactured both in accordance with the ceramic slurry casting process and also in accordance with the pressing process. In order to avoid contamination of the starting material, a zirconium-oxide-containing slurry is used in the casting process. In the pressing process, this slurry or organic

binding materials are employed as binders. In order to avoid contamination of the zirconium material through abrasion of foreign substances, the slurry is produced in a wet mill whose lining consists of shaped elements of zirconium oxide, which elements in suitable shape also perform the function of grinding elements.

The invention is explained on the following exemplified embodiments:

a. Slurry-casting process

A mixture of 83 kg. stabilized zirconium oxide, grain size less than 0.1 mm, and 83 kg. nonstabilized zirconium oxide, grain size less than 0.1 mm, with 34 liters water and 5 ml. aqueous solution of an alkali salt of a polycarboxylic acid, is ground for 200 hours in a wet mill charged with grinding elements of zirconium oxide, and provided with a lining of zirconium oxide bricks. After 200 hours, 60 parts by weight of zirconium silicate, grain size 0.2 -0.5 mm, is added to 40 parts by weight of such a slurry and a mixture is made. The mixture is cast into gypsum molds, removed after 12 hours, dried and fired at 1620°C.

b. Pressing process

In a muller mixer, there are mixed 650 kg. zirconium silicate, grain size 0.2 -0.5 mm, while adding 15 liter sulfite waste liquor (30°B), with 175 kg. stabilized zirconium oxide, grain size smaller than 0.06 mm, and 175 kg. nonstabilized zirconium oxide, for about 10 minutes. The completed mass is pressed on a hydraulic press under 500 kg./cm<sup>2</sup> pressure. The pressed blank is dried and then fired at 1620°C.

The steel-pouring nozzles produced in accordance with this process possess the following properties:

|                           |                  |                 |
|---------------------------|------------------|-----------------|
| Chemical analysis:        | ZrO <sub>2</sub> | 75 % by weight  |
|                           | CaO              | 1.5 % by weight |
|                           | SiO <sub>2</sub> | 20 % by weight  |
| Physical Properties:      |                  |                 |
| Gross density             | 4.0 g/cc         |                 |
| Specific gravity (weight) | 5.0 g/cc         |                 |
| Total porosity            | 20 % by volume   |                 |

When employed in steelworks, the nozzles of the invention withstood the tests of use with excellent results.

I claim:

1. A refractory fired shaped element for closures in casting units for metals, said element comprising 10 to 50 % by weight zirconium oxide and 50 to 90 % by weight zirconium silicate, 30 to 60 % by weight of the total amount of zirconium oxide being present in stabilized form and 70 to 40 % by weight of the total amount of zirconium oxide being present in unstabilized form.
2. A refractory fired shaped element as in claim 1, characterized in that the zirconium oxide is employed in a grain size smaller than 0.1 mm.
3. A refractory fired shaped element as in claim 1, characterized in that the zirconium silicate is introduced in a grain size larger than 0.2 mm.
4. A refractory fired shaped element as claimed in claim 1 wherein the total stabilized and unstabilized zirconium oxide is present at about 35% by weight and the zirconium silicate is present at about 65% by weight.
5. A refractory fired shaped element as claimed in claim 1 wherein the zirconium oxide grain size is smaller than about 0.06 mm.
6. A refractory fired shaped element as claimed in claim 1 wherein the zirconium silicate grain size is about 0.2 -0.5 mm.

\* \* \* \* \*